

## UNITED STATES PATENT OFFICE

2,150,569

TEXTILE MATERIALS AND THEIR  
PREPARATIONWilliam Whitehead, Cumberland, Md., assignor  
to Celanese Corporation of America, a corpora-  
tion of DelawareNo Drawing. Application June 23, 1936.  
Serial No. 86,825

11 Claims.

(Cl. 19—66)

This invention relates to the treatment or preparation of staple fibers which are more suitable for spinning or other textile operations than those heretofore produced.

- 5 An object of the invention is the preparation of anti-static staple fibers, especially those made from or containing organic derivatives of cellulose. Another object of the invention is the treatment and preparation of staple fibers, made from 10 or containing organic derivatives of cellulose, with an anti-static finish wherein the coefficient of friction of the resulting fibers may be controlled, thus permitting the regulation of the drafting of such fibers in spinning operations. 15 A further object of the invention is the preparation of yarns or fibers with an anti-static finish which scours readily from the same in hard or soft water and which does not affect the luster or dyeing properties of the yarns or fibers. Other 20 objects of the invention will appear from the following description.

The formation of "spun" yarn from comparatively short lengths or staples of filaments or threads composed of organic derivatives of cellulose present serious difficulty. This is due to the fact that such organic derivatives of cellulose have a very high di-electric constant and are very poor conductors of electricity, and when the filaments are rubbed together or against machine 30 parts during the various operations involved in mixing, carding, drawing, combing, spinning and like operations, a heavy charge of static electricity is produced. Because of the static electrical charge, the staple fibers containing organic derivatives of cellulose do not adhere to each other readily, tend to adhere to machine parts and cause great difficulty in the textile operations.

I have found that if a mixture of an electrolyte, such as the soaps or salts of amines, a lubricant 40 and a lubricating aid, such as a sulphonated fatty alcohol, is applied to or incorporated with staple fibers containing organic derivatives of cellulose, the tendency to generate static electricity during textile operations is greatly reduced. Moreover, I have found that if such mixture is applied to 45 or incorporated with continuous lengths of artificial filaments, especially those made by the dry or evaporative method of spinning, the great difficulty encountered in winding, drafting, etc., and cutting such filaments to uniform staple lengths is overcome.

For a number of years, solutions of electrolytes in aqueous and non-aqueous solvents have been used as a finish for staple fibers. Although some 50 of these finishes are excellent anti-static finishes,

they usually impart scroopiness and resistance to carding and drafting of the fibers to yarn. Moreover, some finishes are corrosive, particularly if applied in amounts over 1% on the weight of the fiber. In textile operations requiring carding by the woolen, worsted, cut silk or cotton method of forming slivers, rovings, and yarn, it is very essential that the coefficient of friction (i. e. the ease with which the fibers slip over each other) of the fiber be controlled in order that a good drafting may be had and in order that 10 yarns of fine size may be formed from said rovings. By employing the mixture or emulsion of electrolyte in accordance with my invention, the coefficient of friction of the prepared fibers may 15 be controlled such that in either the cotton method, the woolen method or other method of forming yarns, an excellent drafting is attained. The finish produces a lubrication of the fibers sufficient to allow the fibers to slip over one another 20 in drafting operations, permitting the formation of yarns of 30 count or finer measured by the cotton method of measuring yarn.

A further advantage of my invention is that the mixture or emulsion of electrolyte may be applied to fibers consisting of a mixture of woolen or other animal fibers and staple length fibers of organic derivatives of cellulose. The emulsion prepared in accordance with my invention has no deleterious effects upon wool, cotton or silk 30 and does not interfere with textile operations to which the material is subjected. It may, therefore, be applied to mixtures of organic derivatives of cellulose, wool and/or cotton; or it may be applied to staple fibers of organic derivatives 35 of cellulose which are to be mixed with wool and/or cotton. The sulphonated fatty alcohol derivatives have a high softening power and they tend to the finish the advantage of scouring in hard water, which advantage is of particular 40 significance when the organic derivative of cellulose threads are to be blended with wool and subjected to contact with lime soaps.

In accordance with my invention, I treat or 45 prepare staple fibers with a mixture or an emulsion containing an electrolyte such as amine soaps or salts of a sulphonated fatty alcohol or the fatty acids, a lubricant and a sulphonated compound of the fatty alcohol type that acts as an agent in stabilizing the mixture or emulsion, and 50 which acts as a finish for the mixture and a softener for the artificial fibers. By the term "sulphonated fatty alcohol" is meant the fatty alcohols that contain either or both the  $\text{HSO}_3^-$  and/or the  $\text{SO}_4^{2-}$  groups. "Sulphonated fatty al-

cohols", therefore, include the sulphonic acid derivative and the sulphate of the fatty alcohol. The sulphonated compound of the fatty alcohol type also acts as an agent effecting the penetration and uniform covering of the fibers by the mixture or emulsion and for affecting the appearance of the mixture or emulsion in or on the fibers. The lubricant in the emulsion may consist of a mineral oil, vegetable oil, or a part or all 5 of the oil may be replaced by a sulphonated vegetable oil. The mixture or emulsion of electrolyte and lubricant may be incorporated in relatively continuous lengths of artificial filaments in any suitable manner and the continuous lengths may 10 then be cut into staple fibers, or else the staple fibers themselves may be treated with the mixture or emulsion of the electrolyte either during or after cutting, or before any spinning operation, or at any suitable intermediate stage of the 15 spinning operation, or the mixture or emulsion may be applied to the roving, sliver or yarn formed in the fibers.

While this invention is of general application and is applicable to the treatment of natural fibers such as cotton or wool or staples cut from natural silk or yarns or filaments made of reconstituted cellulose (such as may be made by the viscose, cuprammonium or nitrate method), it is 20 of particular importance in connection with staple fibers made of organic derivatives of cellulose such as organic esters of cellulose and cellulose ethers. Examples of organic derivatives of cellulose are cellulose acetate, cellulose formate, cellulose propionate and cellulose butyrate, while 25 examples of cellulose ethers are ethyl cellulose, methyl cellulose and benzyl cellulose. Therefore, 30 this invention will be described more particularly in connection with the preparation or treatment of staple fibers made of cellulose acetate or other 35 organic derivatives of cellulose.

The artificial filaments of organic derivatives of cellulose may be formed from solutions of the same in suitable solvents by extruding said solutions through orifices into a dry or evaporative atmosphere as in dry spinning or by extrusion 40 through orifices into a bath containing a precipitating liquid as in wet spinning. Such filaments may be treated while in the untwisted state by my process, or two or more of such filaments 45 may be associated together by twisting, to form 50 yarns or threads, which yarns or threads may be treated with my process. The mixture or emulsion with which I treat or prepare yarns or fibers 55 may contain from 300 to 350 parts by weight of mineral oil, vegetable oil or sulphonated vegetable oil, or a mixture of these, 20 to 60 parts by weight 60 of a sulphonated fatty alcohol or a salt thereof, which sulphonated fatty alcohol may contain traces of unsulphonated fatty alcohol and from 65 75 to 125 parts by weight of a fatty acid soap of an amine. The sulphonated oils and sulphonated fatty alcohol compounds, in themselves, 70 are anti-static and a mixture of these with the fatty acid soaps of amine would be expected to provide a good anti-static. However, I have discovered that the mixture of these compounds produces a better anti-static finish than either of the compounds separately. Furthermore, the mixture provides a lubricating quality to the yarn and a softening of the fiber which produces fibers 75 having a desirable coefficient of friction for the process.

A further advantage of my invention is that the anti-static qualities are maintained even in cool and dry atmospheres.

The mineral oil employed in forming the emulsion may be any suitable mineral oil, preferably one which is light in color. The mineral oil also is preferably completely saturated. The amount of mineral oil employed as well as viscosity of 5 same will depend to a great extent upon the type of fiber employed and the operation to which the fiber is subjected. For general use in carding, drafting and spinning operations by either the cotton, silk or woolen method of spinning, either 10 where organic derivatives of cellulose fibers are used alone or mixed with wool fibers and cotton fibers, a mineral oil having from 50 to 54 seconds viscosity (Saybolt at 100° F.) is found suitable. However, a mineral oil having a lower or higher 15 viscosity may be employed. In place of some or all of the mineral oil, there may be substituted a vegetable oil such as olive oil, castor oil, etc. In place of either the mineral oil or the vegetable oil, there may be substituted a sulphonated vegetable oil such as sulphonated olive oil, sulphonated castor oil and the like.

The lubricant aid, generally referred to as a sulphonated fatty alcohol, or a salt thereof, may be the sulphonated product of any suitable alcohol, for instance, lauryl, oleyl, stearyl, palmetyl, etc., which sulphonated product contains either or both the sulphonic or sulphate groups. The sulphonated fatty alcohol may contain from a trace to as high as 5% to 10% or more, based on 25 the weight of the sulphonated fatty alcohol, of the free or unsulphonated alcohol. The sulphonated fatty alcohols may be used in the form of their sodium, potassium or amine salts. For instance, the triethanolamine salt of the sulphonated fatty alcohol is found to be exceptionally suited for forming the anti-static finish. In place of employing as a basic material the salt of the sulphonated fatty alcohol, the salt may be formed in the emulsion by adding the base to 30 the emulsion in an amount sufficient to neutralize the acid present. By the term "sulphonated fatty alcohol compound" used in the specification and claims, it is intended to include sulphonated fatty alcohols, the sodium, potassium, triethanolamine, and other salts of the sulphonated fatty alcohols and/or either of the above two compounds or a mixture of same, as well as such compounds that contain from a trace to 10% or more of the unsulphonated fatty alcohol. When 35 it is desirable to form a free flowing anti-static finish suitable for use without the application of heat or agitation, it is preferable to employ the sulphonated fatty alcohol or salt of the lower molecular weight fatty acids such as oleyl alcohol. 40

While any suitable organic electrolyte may be employed, I prefer to employ the hygroscopic organic electrolyte, examples of which are mono-, di-, tri-ethanolamine soaps of fatty acids, the methylamine, aminolamine, etc. soaps of the fatty 45 acids and like amine soaps. The acid part of the soap may be any suitable fatty acid such as oleic, palmitic, stearic, lauric. I have also found that triethanolamine is of exceptional value in mixtures containing the sulphonated oleyl or lauryl 50 alcohol. It is not necessary to use pre-formed soaps of amines as the same may be formed in the mixture or emulsion by adding separately the fatty acid and the amine. The mixture or emulsion of lubricant, electrolyte and aids may be 55 emulsified to any suitable concentration of viscosity by the addition of water. The mixture or emulsion of lubricant can also be applied by warming or heating the mixture if the viscosity of the same warrants it. Where the mixture is 60

emulsified with water, the amount of water employed will depend upon the nature of application to the yarn or fiber and of the textile operation to which the fiber will be subjected.

5 The amount of the individual compounds present in the mixture or emulsion and the amount of the same applied will vary in accordance with the nature of the electrolyte, the lubricant, the nature of the staple fibers and the results to be obtained. Generally, for the cutting and spinning by either the cotton or woolen method of forming yarns, the amount of the individual compounds will be present in about those proportions specified in the example hereinafter given.

10 15 The amount of such mixture applied to or incorporated in the fibers will be from 1% to 10% based on the weight of the fibers, of the substantially water-free emulsion. When the emulsion contains water allowance should be made in the application of the same to the fibers so that upon the evaporation of the water in equilibrium with the atmosphere the desired amount of finish will remain on the fiber. Excellent results have been obtained by the application of from 1% to 3% 20 based on the weight of the fibers of the mixture.

25 The filaments or yarns may be treated with the emulsions of the electrolyte while they are still in the comparatively continuous lengths in which they are formed. Conveniently the emulsion of electrolyte may be applied by means of wicks, rollers or other furnishing devices to the 30 yarn or filaments while they are in transit. A desirable method is to apply the electrolyte emulsion to the artificial silk immediately after the artificial silk leaves the spinning cabinet in which it is formed, while on the way to a cutting device which cuts it into staple fibers. If desired, the relatively continuous lengths may be treated in the form of hanks or other suitable 35 packages prior to being cut into staple or chappe of suitable length. Instead of treating the filaments after their formation with the emulsion of electrolyte, such emulsions may be added to or incorporated in the spinning solution in which 40 said filaments are formed, whereby filaments containing such emulsions are formed directly. The artificial filaments may be formed and if desired lubricated at the metier with any suitable lubricant, then either before or after cutting they 45 may be washed in a bath containing a little soap or other scouring agent and then have a finish containing the anti-static material applied thereto. The washing treatment removes any lubricant that may be present but also removes residual solvent and adds a slight curl to the fiber.

50 Alternatively staple fibers, either natural, such as cotton, wool, or those formed by the cutting of continuous lengths of natural silk or artificial filaments may be treated with the emulsion of electrolyte. In this case the staple fibers may be placed in bags which are immersed in the bath of the emulsion and which, for convenience, may be tied in bundles prior to immersion in the bath. The treatment of the staple fibers may also be 55 made during the intermediate stage of the spinning operation, such as immediately after lapping, carding, drawing, or slubbing. A preferred means of applying the emulsion to staple fibers cut from substantially continuous lengths of 60 filaments containing organic derivatives of cellulose is to spray the emulsion upon the cut fibers as they leave the cutting knives and are blown into a storage space. A still further method of applying the emulsion to fibers is during a mixing or picking operation in which case the emul-

sion is blown, in an atomized form, or sprinkled upon the fibers as they leave the mixer or picker. A still further method of applying the emulsion is in a manner similar to that employed for a long time in the wool method wherein a layer of the fiber is laid upon an oiling floor and the same sprinkled by hand or otherwise with the emulsion and then a further layer laid down and this sprinkled and so on. In the latter method it is preferable to first subject the artificial fibers to 10 a washing or scouring treatment in an aqueous bath containing, for instance from 1 to 10 grams per litre, of soap or other scouring agent.

15 As to the length of the staple fiber, lengths ranging from  $\frac{1}{2}$  or more than 10 inches are suitable. The artificial filaments may be of any suitable weight per unit length, say from 1 to 30 or more denier, examples of which are 1.9, 2.5, 3, or 5 denier or more.

20 After treatment with an emulsion of electrolyte, 20 the short lengths of filaments or fibers are then subjected to a suitable spinning operation, such as those operations used for the spinning of the short lengths of natural silks, cotton or wool fibers to form threads. Any of the well-known 25 systems may be employed to form the yarns or threads, such as the cotton system, the woolen system, the worsted system, the French system, the spun silk system, the Bradford system, etc. These spinning operations also include the preliminary treatments necessary to present the filaments or fibers in the form required for the actual operation of twisting them into yarn. This may include carding, lapping, mixing, spinning, 30 opening up, etc.

35 In order to further illustrate my invention without being limited thereby, the following specific examples are given:

#### Example I

40 A mixture is made by mixing together 312 parts by weight of mineral oil of 50 second viscosity (Saybolt at 100° F.), 28 parts by weight of a sulphonated fatty alcohol, 60 parts by weight of a fatty acid (oleic acid) and 29 parts by weight triethanolamine. These ingredients are mixed until a substantially clear mixture is obtained. Staple fibers, during the cutting operation, are sprayed with this mixture in such an amount that from 1% to 3% on the weight of the fibers of the mixture is applied thereto. The staple fibers are found to be anti-static, softened and lubricated sufficiently to pass through all the textile operations without deleterious effects and be formed by the woolen method of making yarns 45 into a yarn of a finer size than 25 count, by the cotton method of measuring yarns. The mixture is readily scourable in hard or soft water 50 from the yarns.

#### Example II

60 A mixture is made by mixing together 300 parts by weight of sulphonated olive oil, 30 parts by weight of a sulphonated alcohol and 90 parts by weight triethanolamine oleate. A small 65 amount of triethanolamine is added to neutralize any developed acidity. The staple fibers are sprayed with this mixture in such an amount that from 1% to 3% on the weight of the fibers of the mixture is applied thereto. The staple fibers are 70 found to be anti-static, softened and lubricated sufficiently to pass through all the textile operations without deleterious effects and be formed by the woolen method of making yarns into a yarn of a finer size than 25 count, by the cotton method 75

of measuring yarns. The mixture is readily scourable in hard or soft water from the yarns.

To any of the mixtures made in accordance with the above descriptions, there may be added a small amount, for instance, from 1% to 20% on the weight of the mixture, of an organic hygroscopic agent, which agent is a softening agent for organic derivatives of cellulose. These agents may be the glycols and/or their ethers.

It is to be understood that the foregoing detailed description is given merely by way of illustration and that many variations may be made therein without departing from the spirit of my invention.

Having described my invention, what I desire to secure by Letters Patent is:

1. In a method of forming spun yarns containing short lengths of fibers of an organic derivative of cellulose, the steps of incorporating therewith before the drafting operation a mixture of an organic electrolyte comprising a fatty acid soap of an amine, a lubricant and a sulphonated fatty alcohol compound and then spinning the treated fibers into a yarn.

2. In a method of forming spun yarns containing short lengths of fibers of cellulose acetate, the steps of incorporating therewith before the drafting operation a mixture of an organic electrolyte comprising a fatty acid soap of an amine, a lubricant and a sulphonated fatty alcohol compound and then spinning the treated fibers into a yarn.

3. In a method of forming spun yarns containing short lengths of fibers of an organic derivative of cellulose, the steps of incorporating therewith before the drafting operation a mixture comprising an organic electrolyte, a lubricant and a sulphonated fatty alcohol compound and then spinning the treated fibers into a yarn.

4. In a method of forming spun yarns containing short lengths of fibers of cellulose acetate, the steps of incorporating therewith before the drafting operation a mixture comprising an organic electrolyte, a lubricant and a sulphonated fatty alcohol compound and then spinning the treated fibers into a yarn.

5. In a method of forming spun yarns containing short lengths of fibers of an organic derivative of cellulose, the steps of incorporating therewith before the drafting operation a mixture comprising an organic electrolyte, a lubricant comprising one or a mixture of the compounds selected from the group consisting of mineral oil, vegetable oil and a sulphonated vegetable oil, and a sulphonated fatty alcohol compound and then spinning the treated fibers into a yarn.

6. In a method of forming spun yarns containing short lengths of fibers of cellulose acetate, the steps of incorporating therewith before the drafting operation a mixture comprising an organic electrolyte, a lubricant comprising one or a mixture of the compounds selected from the group consisting of mineral oil, vegetable oil and a sulphonated vegetable oil and a sulphonated fatty alcohol compound and then spinning the treated fibers into a yarn. 10

7. In a method of forming spun yarns containing short lengths of fibers of cellulose acetate, the steps of incorporating with the fibers before the drafting operation a mixture comprising from 300 to 350 parts by weight of a lubricant, 15 from 75 to 125 parts by weight of an organic electrolyte and from 20 to 60 parts by weight of a sulphonated fatty alcohol compound and then spinning the treated fibers into a yarn.

8. In a method of forming spun yarns containing short lengths of fibers of organic derivatives of cellulose, the steps of incorporating therewith before the drafting operation a mixture comprising an organic electrolyte, a lubricant, a sulphonated fatty alcohol compound and an organic hygroscopic material and then spinning the treated fibers into a yarn. 25

9. In a method of forming spun yarns containing short lengths of fibers of cellulose acetate, the steps of incorporating therewith before the drafting operation a mixture comprising an organic electrolyte, a lubricant, a sulphonated fatty alcohol compound and an organic hygroscopic material and then spinning the treated fibers into a yarn. 30

10. In a method of forming spun yarns containing short lengths of fibers of organic derivatives of cellulose, the steps of incorporating in said fibers before the drafting operation a mixture comprising an organic electrolyte, a lubricant and a sulphonated fatty alcohol compound, said step of incorporation of the mixture with the fibers being performed while the mixture is at an elevated temperature and then spinning the treated fibers into a yarn. 40

11. In a method of forming spun yarns containing short lengths of fibers of cellulose acetate, the steps of incorporating in said fibers before the drafting operation a mixture comprising an organic electrolyte, a lubricant and a sulphonated fatty alcohol compound, said step of incorporation of the mixture with the fibers being performed while the mixture is at an elevated temperature and then spinning the treated fibers into a yarn. 50

WILLIAM WHITEHEAD. 55